

Nov. 14, 1939.

A. W. MORRIS

2,179,513

## METAL CASTING

Filed April 12, 1935

2 Sheets-Sheet 1



*Inventor*  
Albert W. Morris  
*By* Nathaniel Frucht  
his Attorney

Nov. 14, 1939.

A. W. MORRIS

2,179,513

METAL CASTING

Filed April 12, 1935

2 Sheets-Sheet 2



Inventor  
Albert W. Morris  
By  
Nathaniel Trucht  
his Attorney

## UNITED STATES PATENT OFFICE

2,179,513

## METAL CASTING

Albert W. Morris, Springfield, Mass., assignor to  
 Morris Engineering Corporation, a corporation  
 of Rhode Island

Application April 12, 1935, Serial No. 15,939

2 Claims. (Cl. 22—188)

My present invention relates to the art of casting metals, and has particular reference to the production of better castings at lower cost.

The present practice in casting metals includes the use of sand or metal molds, and a furnace in which the metal to be cast is melted, the molten metal then being conveyed in ladles from the furnace to the molds and poured therein. The castings, when cooled, are sandblasted or tumbled, and then machined.

The problem of producing better castings comprises selection of the metal which is most suitable for the desired casting, casting of this metal under the most suitable conditions, and use of a mold which does not change or effect the character of the casting or its surface whereby the completed casting has a smooth, unblemished surface, and requires little or no finishing or machining.

20 The principal object of my invention is to produce castings having ideal chemical and physical characteristics.

An additional object of my invention is to perform the casting operation under the conditions 25 most suitable for the metal being cast.

A further object of my invention is to utilize a mold that is inert or has a definite predetermined reaction to the cast metal.

Another object of my invention is to provide a 30 smooth cast surface that is unblemished and does not require finishing.

A still further object is to obtain a finished casting of accurate, predetermined size.

With the above and other objects and advantageous features in view, my invention consists of novel arrangements of parts, and novel methods of casting, more fully disclosed in the detailed description following, in conjunction with the accompanying drawings, and more specifically defined in the claims appended thereto.

In the drawings:

Fig. 1 is a front elevation, partly in section, of a novel casting furnace;

Fig. 2 is a central transverse section thereof; and

Fig. 3 is a perspective of a novel mold section.

The casting of metals has heretofore been handled as follows: The metal has been melted within a furnace where the atmosphere in contact with the metal bath has been suitable for the particular metal, as in an open-hearth, air, or electric furnace. The molten metal has then been "tapped" and taken from the furnace to the molds, and the desired pieces cast by pouring the metal into the molds.

In practice I have found the following objections to this common method. When the metal is taken from the furnace it cools rapidly before being poured for castings; to offset this the metal is superheated, which is costly and is bad metallurgically, whereby the metal is not ordinarily maintained at the best casting temperature for the desired metallurgical results in the casting, and the castings are not uniform. Moreover, the pouring temperature for different castings varies widely. But perhaps more important than the difficulty due to wide variation in temperatures between the furnace and the molds is the common difficulty of varying atmospheric conditions. When the metal is taken from the furnace in a ladle it is soon exposed to and contaminated by the outside air both before pouring and as the metal is poured into the molds; moreover, the molds are full of gases and air that also contaminate the metal poured into their cavities, as do also the cold surfaces of the molds. These difficulties have not been entirely overlooked; I am aware that much work has been done to improve the methods of handling hot metals between the furnaces and the molds and to prepare the molds for receiving the metal. But so far as I know, such improved methods are expensive and the results have not yet been satisfactory for metals melting at very high temperatures like steel, for in one way or another such metal is contaminated more or less during the transition time between furnace and mold or in the mold, and such metal is particularly susceptible to contamination by exposure to an atmosphere other than one specially prepared for the particular metal.

This is particularly true of metals melting at very high temperature—2000° F. and above, which commonly need to be poured as the molds are being filled. I am aware of casting methods in which the molds are filled by suction action or by pressure causing mold filling movement of metal from a suitable reservoir. Without going into the distinctions in detail, one skilled in the art knows that these prior casting methods are not suitable for general application; they are expensive; and they have not and apparently cannot be used in a great many places where the casting molds must be filled by the metal pouring methods as distinguished from suction, pumping, or immersion methods, as in many instances the expense is too great. But with metals at temperatures about 2000° F. substantially all casting is done by metal pouring methods to fill the molds.

According to my invention I can pour the metal in the usual way to fill the mold, but I eliminate the time element in the present practice of transferring the metal from the furnace to position 5 for pouring it into the molds. To do this I carry the mold to the melting furnace, insert it in the furnace, pour the metal to fill the mold while both mold and metal are in the furnace, and then either remove the mold with its casting from the 10 furnace, or I may remove the casting from the mold while it is still in the furnace. In such operations there is a time element in the step of pouring the metal from the molten mass to fill the mold; with my mold filling method the pouring 15 takes place while the mold is in the furnace and the operation is possible without using any time during which the molten metal is in transit between the furnace and any point outside of the furnace, and without exposing the metal 20 while being poured to an atmospheric condition different from that in the furnace. The metal is put in the mold before the mold leaves the furnace, and in its cast condition the metal is taken from the furnace either with or without the 25 mold, as explained hereinafter. Thus, there is no chance for contamination of the molten metal by transporting it between the furnace and the mold, and yet the mold is filled by the desired and simple pouring step as from a ladle. Furthermore, 30 by inserting the mold into the melting furnace prior to the ladle pouring operation, the interior mold surfaces and the cavities formed by them are prepared in an effective way for taking the hot metal under the best conditions. The extremely high temperature of the furnace 35 will act instantly on said surfaces to dry them; and will also act instantly on all the gases carried in the mold cavities to expand these gases and drive them out of the mold. So before the mold can be filled these cavity gases (which cause so much trouble in the present casting practices) are driven out and dissipated in the much larger body of gases above the molten mass of metal whereby the cavity atmosphere 40 before pouring will be substantially the same as the furnace atmosphere above the molten mass. That atmosphere is normally and suitably controlled according to the character of molten metal mass and is one that does not contaminate the metal; in other words, it is inert to the molten metal. It is an entirely different atmosphere than obtains in the mold cavities and against the surfaces of the metal as treated in the present casting practice where the metal is 45 carried from the furnace and poured from a ladle to the mold.

My method may be carried out in practice by labor saving apparatus of various kinds co-ordinated for the purpose, but it may be carried 60 out by hand operations, and I want to emphasize that no expensive apparatus is needed.

Referring to the drawings, I may melt the metal, stainless steel for example, in an open-hearth furnace represented in the drawings by 65 the reference numeral 10. The melted metal rests on the hearth 11 and is at very high temperature when ready for casting, but need not be superheated. A characteristic of stainless steel 70 is that given any opportunity it will absorb carbon with great avidity; it is an alloy and the less carbon it contains the less proportion of expensive elements is necessary in the alloy to give the stainless results. It is also susceptible to 75 contamination in other respects. This is one

reason that stainless steel castings made in the ordinary way are frequently defective.

I leave the molten body of stainless steel in the furnace and do my casting in the furnace. The open-hearth furnace has an atmosphere of hot gases passing over the surface of the melted bath; the gases are controlled so that the composition of the alloy will remain as wanted in the casting. Furthermore, these furnace gases maintain the desired temperature in the liquid, such temperature of the metal being easy to regulate when it is in a large mass and kept in the furnace. I make use of this situation by holding the temperature and atmosphere above the furnace metal at the points best suited to casting. Ordinarily 15 the furnace temperature needs to be kept far above the best casting point so as to compensate for the loss of heat when the metal is transported from the furnace to the molds, and when thus transported the metal is commonly poured in an atmosphere and at a temperature, both outside and inside the mold, that are not so good as the furnace atmosphere and temperature.

Referring to Figs. 1 and 2, I prefer to provide a ladle 12 inside the furnace, pivotally mounted on a bar 13 which may be rotated by a handle from outside the furnace. An endless chain conveyor 14 which may be stopped at any point, by any suitable control mechanism, passes through the aligned doors 15, 16 of the furnace, and may 30 pass below the furnace, but preferably extends over the top, thus affording a three point support by means of gears 17, 18, and 19 at the support points, one of the gears being motor driven. A plurality of book type molds 20, see Fig. 3, each 35 comprising a mold section 21 and a check section 22, are hingedly mounted in the conveyor and are adapted to be closed by a U-shaped plunger 23, and to be retained in closed position by a manually applied clamp 24; as the molds pass the 40 ladle 12, they are stopped, the ladle is tilted to fill the molds, and the molds move out to the agitator 25, where the clamp is removed, the agitation opening the molds to permit removal of the 45 castings. A second U shaped plunger arrangement 23 may be utilized to control the speed of opening of the molds. The ladle is hand filled by dipping into the molten metal, but may if desired be filled by means of an endless bucket arrangement. Any known type of releasable 50 spring connection may be used for the conveyor and the molds to keep the molds open until closed as described.

The advantages in filling the mold by pouring the metal as described above are that its surfaces and cavities are nicely prepared by the heat of the furnace for receiving the casting, the time for the molten metal to leave its furnace body and get into the mold is brought to a minimum, and the exposure of the metal as it is being 55 poured is in the atmosphere of the furnace gases and at the same temperature, with minimum risk of contamination. The pouring from ladle to mold can take place without any danger of pouring too much as all excess drops immediately to 60 the furnace bath, so that wastage or expense of remelting is avoided; the mold may if desired be made to take this into account as by having exit passages to cause a mold circulation of hot metal until its cavities are filled solidly. But the most 65 important advantage resides in the ideal conditions surrounding the pouring operation for the transfer of metal from the body in the furnace to the cavity in the mold, without contaminating 70 exposure to atmospheric or cold body surfaces 75

of the mold such as occur in the present mold pouring practice.

In using my method for making malleable castings there is a further advantage in that my molds 5 may be moved directly from the furnace where they are filled to the annealing furnace in which the mold may be emptied and the casting annealed with a minimum heat loss; and the less handling between the melting furnace and the 10 annealing furnace, the better their metallurgical character can be safeguarded. The method can be used with the air type of furnace as well as the open-hearth, and in the same way.

The operation of my method with regard to the 15 electric furnace is essentially the same as in the case of the open-hearth furnace, with this and possibly additional advantages. A well known type of electric furnace is of the rocking type; as the furnace rocks in its normal operation for temperature transfer, the molten mass can be picked up by a pouring lip and the mold filled by the movement of the furnace as the mold is stopped within the furnace. One advantage in the use of an electric furnace resides in the better control of the atmosphere therein.

It will be of advantage in some instances to remove the castings while still in the furnace. This can be provided for by a shelf, not shown, at the side of the hearth where the casting can be left. And it will be advantageous in some instances to pass the castings as they are removed from the furnace through a furnace door directly into an annealing oven. One of the doors may be in a passage from the furnace to an annealing 35 oven and opened to admit the casting from the furnace, the advantage residing in the elimination of contaminating influences.

Stainless steel, malleable iron, grey iron, ordinary steel, and such very high melting point 40 metals may readily be cast by pouring the metal under this method. By "stainless steel" as used in this specification I mean to include all the steel and iron alloys which are important from their characteristic in resisting rust and acid. Alloy steels and irons of the class included are 45 known by various names popularly called stainless steel but which include such metals as rustless iron, Silchrome, Invar, Durimet, and trade names now well known but which vary from time to time.

Malleable iron may be cast as described, with great increase in strength and quality, and at a great saving in cost. The production of malleable 50 cast iron comprises, first, the production of white iron castings which are hard and brittle, and second, the annealing of the white iron castings to obtain a ductile product, this annealing changing the "combined" carbon in the casting to "free" carbon, technically known as "temper" carbon. The character of the casting depends on the composition and its uniformity, and the air furnace is used in the United States for high 55 grade malleable, instead of the cupola, to increase the uniformity; the open hearth furnace is used in Europe, for the same reason.

The properties of malleable iron are largely controlled by the amount of carbon present, which may be as low as 2.00% or as high as 3.00%. High carbon in general makes the metal weak and 60 less ductile, but produces sound machineable castings of good surface; with high carbon, the silicon is ordinarily kept low to obtain best results in the neighborhood of .50% to .60% and conversely, is kept high, to as much as 1.20% to 1.30% with low carbon iron. If high carbon,

high silicon are both used as with the present practice, the poured metal, using sand molds, will not be white as the carbon separates and becomes free as the temperature drops. The manganese and sulphur vary together, from .25% to .49% for manganese, and from .05% to .14% for sulphur; phosphorous is preferably below .20% and may be less than .10%.

With the improved casting method, it is feasible to cast malleable iron having both high carbon and high silicon, thus obtaining greatly improved tensile and other physical characteristics, and quicker annealing, while retaining the desired white fracture, which shows that all the carbon is combined. Thus, when using a typical 15 malleable iron having the following analysis:

|    | Per cent |
|----|----------|
| C  | 2.75     |
| Si | .65 20   |
| Mn | .30      |
| S  | .07      |
| P  | .20      |
| Fe | Balance  |

the tensile strength was determined to be 54,000 25 lbs. per sq. inch, the elongation in two inches, 18% and the reduction in area 18%.

When using a malleable iron as follows:

|    | Per cent      |
|----|---------------|
| C  | 2.75 to 3.00  |
| Si | 1.20 to 1.50  |
| Mn | .30 to .70    |
| P  | .05 to .10    |
| S  | .05 to .10 35 |

the tensile strength became 70,000 lbs. per square inch, the elongation 24% and the reduction in area 25%.

The cost was also greatly reduced; casting time was cut 50%, annealing time was reduced 40 25%, tumbling and sand blasting were eliminated, and the required machining was less.

Having described how I obtain a casting of metal under ideal conditions, I will now explain how a casting having a smooth, unblemished surface may be obtained by utilizing a metal mold which is inert to the cast metal, with particular reference to the casting of stainless steel as an example.

Stainless steel as cast in the usual way comes out of the mold with a rough surface where the sand has adhered, or a crust of blemished metal. When a smooth finish is needed, the rough surface or crust is cut or ground off to expose the unblemished and permanent surface often desired for ornamental purposes and sometimes for machine parts that are wanted in finished forms and with finished surfaces. So far as I know, stainless steel shapes have not heretofore been cast without the crust that must be cut off to expose the ornamental character of the metal.

According to one feature of my invention, I make stainless steel castings that do not need to have their surfaces cut off to expose the ornamental character of the metal.

Stainless steel castings have heretofore been made in sand molds and not in permanent molds, the reason being that permanent molds have ingredients that react chemically on the stainless steel. The latter is peculiarly susceptible to chemical changes at the very high temperature at which the metal must be cast; it is an alloy, the elements of which have an avidity at the high casting temperature for most other elements. This makes the casting of stainless steel 75

difficult. It seems to be true from experience that when cast in sand molds, stainless steel will retain its chemical integrity except for the forming of the crust above mentioned.

According to my invention, I not only make stainless steel castings with their ornamental surface, but do this in a permanent mold. The fact that I have discovered a way to make good stainless steel castings at a greatly lowered cost 10 compared to known methods, has special significance.

Everyone knows that stainless steel would have a much wider use in making cast shapes if it were not so high in cost. One skilled in the art 15 knows that the prohibitive cost is primarily due to the surface finishing operation, rather than the cost of the alloy metal itself, although the latter is expensive. Many shapes that are wanted in stainless steel form are not commercially available on account of the expense; for example, an ornamental door knob for an automobile can be made of easily cast metal and chromium plated at a much less cost than the same piece can be made of stainless steel surface 20 by prior art methods. So the plating method is used commercially because the stainless steel surface in that shape would be too expensive to obtain.

My invention is particularly aimed at increasing 30 the uses of stainless steel shapes under these competitive conditions.

To practice my invention I proceed as follows: I provide a permanent mold of metal lined 35 with copper, the copper being alloyed with a hardener such as aluminum to toughen it and make it easier to cut the mold cavity, see Fig. 3, the mold sections 21, 22 having the described lining 26. The mold may be entirely of copper and aluminum, and is made of sufficient bulk 40 to absorb the heat of the cast metal and avoid fusing the mold surfaces. This will follow as a result of the high heat conductivity of the mold, which takes the heat from the molten steel so fast that the temperature at the molding surfaces is not high enough over a sufficient time 45 to melt the mold. This characteristic of my mold enables me to use copper alloyed with aluminum even though such alloy will melt far below the melting point of any steel.

In making the mold for my purpose I select 50 copper as its principal metal, which gives me the characteristic above mentioned. The addition of aluminum acts as a hardener to facilitate machining the mold and other handling.

In a general sense a copper mold used for casting steel will not contaminate the chemical characteristics of the steel. The metal of the mold is generally inert chemically to an ordinary steel metal being cast. By being generally inert, I 55 mean that the body of one will not be affected by the body of the other in the wandering of chemical constituents from one to the other in the casting operation at the relative temperatures of contact. But in casting stainless steel 60 I have discovered that this general inert condition is not all that is desirable to safeguard the casting against surface contamination. The surface of the casting in a stainless steel article is the thing my invention is particularly intended 65 to make right and uniform in great numbers of castings from the same mold.

I have found that, although in extremely small quantities, there is enough migration of elements between ordinary copper and stainless steel at 70 75 the casting temperature to contaminate the sur-

face of the castings in repeated use of the mold. It is not ordinarily perceptible, so far as the bodies of the metals are concerned, but is perceptible in the surface appearance of the stainless steel. And that is what I want to safeguard. 5

I have discovered that this slight migration of elements may take place in either direction, from the stainless steel to the mold or vice versa, and either way it affects the surface. If the mold takes the elements from the hot metal, 10 successive castings have a tendency to stick. If the hot metal takes elements from the mold, the mold surfaces are eaten away.

When I state that there is a migration of constituents between the metals in contact at casting temperature, it should be understood that I am speaking about such small quantities as would not ordinarily affect the body of either metal appreciably. In that sense the bodies of the two metals may be chemically inert as they contact. But they are not chemically inert with respect to such small migration as will mar the surface appearance of stainless steel if it absorbs material from the mold.

Thus, the stainless steel has an affinity for 25 carbon, and will take carbon from the mold surface, if present. Copper and aluminum have affinities for some of the metals of the stainless steel composition, and will draw these metals from the case metal surface. I have therefore 30 added enough iron, nickel, silicon and chromium to the mold material to satisfy this affinity, whereby there is substantially no migration of metals from the stainless steel to the mold, and the surface of the cast stainless steel is smooth, 35 clean and unblemished. Preferably, the amounts of the satisfying metals added are set so as to obtain a slight tendency to migration from the cast metal to the mold.

I have not thought it necessary to give exact 40 constituents of my mold invention as they may vary considerably in practice, and according to the character of stainless steel to be cast. The skilled metallurgist will know how to proceed from my disclosure. He will consider the subject of what metals will migrate between such casting metal and a copper mold. He will then alloy the copper from the mold so as to provide a definite but very small overbalance to direct the migration from stainless steel constituents to 50 mold constituents. He need not try to get an exact balance of chemical inertness (a difficult matter) because even if he should succeed in that way with respect to one mold and one melt of stainless steel, the next melt of stainless steel might throw out the balance and migration might be in the direction of the casting metal and mar the desired stainless surface. And when the constituents of the steel are changed (there being considerable variation possible in stainless 55 steel) the mold work in the assumed case would be uncertain and not uniform. But by proceeding as I have disclosed herein, the alloyed copper mold can bring out the right surface in the stainless steel in a uniform casting manner with 60 great economy in any desired shapes and in commercial quantities under a uniform practice. In this way many stainless steel shapes not heretofore commercially available are now 65 made so. The extra cost of the stainless steel metal is small in comparison with the cost of the eliminated surface finishing operations.

For illustrative purpose I am disclosing the following example of mold and stainless steel constituents that may be used as disclosed or 70 75

deliberately varied for the purposes of practicing my invention:

*Examples*

1. Metal:

|            | Per cent by weight |
|------------|--------------------|
| Carbon     | .80-.16            |
| Manganese  | .30-.50            |
| Silicon    | .20-.40            |
| Chromium   | 17.00-18.00        |
| Nickel     | 9.00-10.00         |
| Sulphur    | .025               |
| Phosphorus | .025               |
| Iron       | Balance            |

2. Mold:

|    |          |      |
|----|----------|------|
| 15 | Copper   | 88.0 |
|    | Aluminum | 8.0  |
|    | Iron     | 1.0  |
|    | Chromium | 1.0  |
|    | Silicon  | 1.0  |
| 20 | Nickel   | 1.0  |

The described mold is best suited for stainless steel castings; I have found, however, that an inert or a substantially inert mold can be determined for any cast metal, and that a satisfactory base is copper having a small percentage of hardener metal alloyed therewith. Thus, for casting malleable iron, the mold should com-

prise copper, a hardener such as aluminum, and a small fraction, in the neighborhood of 1%, of Fe, to saturate the aluminum in the mold, and thus eliminate migration. The addition of migration control ingredients depends on the particular cast metal and may be omitted for grey cast iron and malleable iron.

While I have described the casting of metals under furnace conditions, and the use of molds having inert characteristics with respect to the cast metals, whereby smooth, unblemished castings of very high quality are obtained, it is obvious that changes in the apparatus and the methods described, to meet the requirements for casting different metals, may be made without departing from the spirit and the scope of the invention as defined in the appended claims.

I claim:

1. In the casting of malleable iron, the steps of pouring the metal into a mold consisting principally of copper and approximately one per cent of iron.

2. A metal mold for the casting of malleable iron, consisting principally of copper and containing iron the amount of iron being less than two per cent and more than one-half of one per cent.

ALBERT W. MORRIS.